

# UNITED STATES PATENT OFFICE.

GOHEI IWATSUBO, OF KYOTO, JAPAN.

## PROCESS OF MANUFACTURING PAPER LEAVES.

1,307,404.

Specification of Letters Patent. Patented June 24, 1919.

No Drawing.

Application filed April 23, 1917. Serial No. 164,056.

To all whom it may concern:

Be it known that I, GOHEI IWATSUBO, manufacturer, a subject of the Emperor of Japan, residing at No. 24 Hontoro-Machi, 5 Takakura-Nishi-Iru, Matsubara-Dori, Shimo-Kio-Ku, city of Kyoto, Empire of Japan, have invented certain new and useful Improvements in Processes of Manufacturing Paper Leaves, of which the following 10 is a specification.

This invention relates to improvements in a method of finishing paper leaves, and particularly to a method in which paper is to be coated with a substance imparting to the 15 paper a desirable finish and permitting the embossing or shaping of the paper so as to render the same suitable for use in artificial flowers and the like.

In the known method of finishing paper 20 for this purpose it has been customary to coat the unfinished paper with a mixture of glycerin and gelatin to which a suitable pigment or die had been added. After the application of this mass to the paper the same 25 was subjected to an embossing or punching operation, the dies having been heated and being applied to the unfinished, or rear, surface of the paper. The disadvantage of this method was that in the embossing or 30 pressing operation portions of the coating dropped off the finished surface of the paper, so that this method resulted in considerable waste of material.

It is an object of the present invention to 35 avoid this waste and disadvantage by adding to the substances of which the mixture is formed an additional substance which imparts to the mixture the desired adhesiveness, avoiding thereby the separation of 40 parts of the coating from the paper surface.

In the known method of finishing paper 45 for the purposes stated, a film of gelatin was applied to the leaf, and this film was then covered with glycerin containing a pigment, as, for instance, white zinc, when it was desired to finish the paper in white. The application of the glycerin to the gelatin film

sometimes produced a coating which cracked or dropped off or was forced off in the embossing operation. 50

According to the present method, a mixture is made of the following ingredients, in the proportions stated:

|                           |       |    |
|---------------------------|-------|----|
| Gelatin                   | 3.2%  | 55 |
| Glycerin                  | 1.4%  |    |
| White zinc or zinc flower | 38.5% |    |
| Magnesium carbonate       | 12.8% |    |
| Calcium chlorid           | 0.6%  |    |
| Water                     | 38.5% | 60 |

The addition of the small amount of calcium chlorid to this mixture is sufficient to impart to this mixture the desired adhesiveness, so that even after the embossing operation the coating will remain on the paper 65 leaf and will form a film thereon, eliminating the danger of cracking or dropping off. The calcium chlorid forms a solvent for the glycerin and prevents the premature evaporation of the moisture in the glycerin, so 70 that all of the substances contained in the mixture remain in that pasty condition in which it is desired to have them for the purpose of effecting the pressing or embossing. Other solvents, as alkaline hydrates, may be 75 used together with the other ingredients of the film forming material.

When the calcium chlorid is heated to about 200° centigrade, the water contained in the mixture will be entirely evaporated 80 without, however, depriving this mixture of its pasty consistency, which is necessary to make the impressions produced by the die upon the paper permanent impressions. This characteristic quality of the entire 85 mass is not impaired even if the dies for the embossing operation or for the pressing are heated. Upon application of the heated dies to the paper, the glycerin and gelatin, owing to the presence of the calcium chlorid, are 90 again softened, if they should have become dry, and the entire mixture will then adhere to the paper and will not be transferred to that material which frequently is interposed

between the dies and the surface to be finished.

Instead of the white zinc other pigments may be used for the film described.

5 What I claim is:

A method of preparing paper for embossing, which consists of applying a coating of a mixture of gelatin, glycerin, pigment, and calcium chlorid to the surface of paper

and applying a hot die to the paper treated 10 in this way.

In testimony whereof I affix my signature in presence of two witnesses.

GOHEI IWATSUBO.

Witnesses:

W. EBITARAH,  
I. SUKUR.